

M. C. ST. JOHN,  
ELECTROPLATED PROPELLER FOR AERIAL VEHICLES,  
APPLICATION FILED FEB. 18, 1920.

1,385,802.

Patented July 26, 1921.



Witnesses

Rudolph J. Berg

Charles F. Fogg.

Inventor

MILES C. ST. JOHN.

By Charles F. Fogg, Atty.

# UNITED STATES PATENT OFFICE.

MILES C. ST. JOHN, OF CHICAGO, ILLINOIS, ASSIGNOR OF ONE-HALF TO JAMES ERICKSON, OF CHICAGO, ILLINOIS.

## ELECTROPLATED PROPELLER FOR AERIAL VEHICLES.

1,385,802.

Specification of Letters Patent. Patented July 26, 1921.

Application filed February 18, 1920. Serial No. 359,523.

To all whom it may concern:

Be it known that I, MILES C. ST. JOHN, a citizen of the United States, and a resident of the city of Chicago, in the county 5 of Cook and State of Illinois, have invented certain new and useful Improvements in Electroplated Propellers for Aerial Vehicles; and I do hereby declare that the following is a full, clear, and exact description 10 of the same, reference being had to the accompanying drawings, and to the numerals of reference marked thereon, which form a part of this specification.

This invention relates to an electroplated propeller for aerial vehicles and process of making the same. Airplane propellers of the type ordinarily used are constructed of wood and on account of the great strength needed the wood which is used in the construction must be the very best. These wooden propellers are carefully formed and finished by hand and their manufacture is an expensive process. After the wooden propeller is finished and balanced by hand, 20 the problem of protecting the surface thereof from the weather arises. This problem has proven to be a serious one and heretofore no really satisfactory method has been devised for completely protecting the airplane propeller from the ravages of the weather. Slight imperfections in the varnish causes checking and cracking to set in and when the varnish is damaged moisture is allowed access to the propeller wood and 30 the propeller is soon rendered useless.

It is an object, therefore, of this invention to provide a propeller for aerial vehicles the surface of which is protected by a coat of metal deposited thereon by an electrolytic process.

It is also an object of this invention to provide an electroplated airplane propeller.

It is another object of this invention to provide a process of making a propeller for aerial vehicles wherein the propeller is formed of wood pulp to the approximate shape desired, a protecting coat of metal deposited on the surface thereof by an electrolytic process and balancing of the propeller effected by further deposition of metal by an electrolytic process on certain portions thereof.

It is a further object of this invention to provide a propeller for aerial vehicles which 55 is formed from pressed fibrous material and

protected and strengthened by a coat of metal deposited on the surface thereof by an electrolytic process.

Other and further important objects of this invention will be apparent from the disclosures in the specification and the accompanying drawings.

The invention (in a preferred form) is illustrated in the drawings and hereinafter more fully described.

On the drawings:

Figure 1 is a view in front elevation of an electroplated propeller for aerial vehicles embodying the principles of this invention.

Fig. 2 is a section on line 2—2 of Fig. 1, 70 showing the interior or body of the propeller constructed of pressed fibrous material.

Fig. 3 is a section on line 3—3 of Fig. 1 showing the pressed fiber construction.

As shown on the drawings:

The propeller of this invention comprises in general the blade portions 1 and the hub 2, both of which portions are covered by a coating of electrolytically deposited metal 3. Said coating 3 is preferably formed from 80 some non-corrosive metal such as copper, although any metal that is desired may be used. In the manufacture of the airplane propeller of this invention, the wooden or fibrous interior portion is first shaped to 85 approximately the form desired. The surface of said interior portion is then prepared for the process of electroplating by a thorough application of graphite or plum-bago to the surface thereof.

The metal to be deposited and the prepared propeller are next deposited in a solution of electrolyte, as, for example, copper sulfate. In this electrolytic process the metal constitutes the positive electrode and the prepared graphited propeller constitutes the negative electrode. Said electrodes are connected together by a conductor of electricity and a source of direct current such as a storage battery or electrical machine is 100 connected in the circuit. Due to the well-known process of electrolysis, the copper from the positive metal electrode will be deposited on the graphited propeller or the negative electrode. This process of deposition of metal will cover the surface of the propeller far more thoroughly than would be possible by the use of varnish applied either by dipping or by manual means. The surface of the propeller is covered so 110

thoroughly that neither air nor moisture can gain access thereto. The metallic covering 3 may be built up to any thickness desired by said process of electrolytic deposition and thus may be used to add strength and rigidity to the propeller. This fact makes possible the forming of the interior portion of the propeller from pressed fibrous material such as wood pulp, a feature which is particularly important due to the increasing scarcity of suitable timber for airplane propellers. The edges of the propeller blades 1 may also be built out to any form desired by this process of electrolytic deposition, and if such edges are subsequently injured by accident or otherwise they may be easily repaired by depositing metal thereon. It may also be clearly seen that balancing of the propeller may be very exactly and effectually accomplished by this process of electrolytic deposition.

By this process it is also possible to cover the main portions of the blades and the hub with one metal and to build out the tips of the blades with another metal.

As may be clearly seen from the foregoing description, this invention provides an effective method of protecting airplane propellers from the weather. In addition, the metal covering provided adds rigidity to the propeller and makes possible the construction from stamped fibrous material, as heretofore described.

Balancing of the propeller and building up of the edges and tips of the blades is much more effectually and economically accomplished than heretofore possible.

The process of this invention provides an economically constructed propeller for aerial vehicles the life of which is practically indefinite. Damaged propellers can be easily repaired and rebalanced by the process of electrolytically depositing metal. This constitutes a great superiority over the old type of wooden propellers where slight damage is irreparable and the damaged propeller must be replaced by a new one.

I am aware that numerous details of con-

struction may be varied through a wide range without departing from the principles 50 of this invention, and I therefore do not purpose limiting the patent granted otherwise than necessitated by the prior art.

I claim as my invention:

1. A propeller comprising a core of pressed 55 fibrous pulp, and an electroplating of metal.

2. A propeller comprising a core of pressed fibrous pulp, an electroplating of metal and at the required points an additional electroplating of metal. 60

3. The process of making a propeller which consists in pressing a fibrous pulp to the form of a core, coating said core with a substance capable of receiving an electrodeposit of metal, electroplating said coated 65 core with metal and balancing the propeller by electrodepositing additional metal at the requisite points.

4. The process of making a propeller which consists in pressing a fibrous pulp to 70 the form of a core, electroplating said core with metal and balancing the propeller by electrodepositing additional metal at the requisite points.

5. The process of making a propeller 75 which consists in pressing a fibrous pulp to the form of a core, electroplating said core with metal and balancing the propeller by electrodepositing additional metal at the requisite points, different kinds of metal being 80 used for coating different parts of said propeller.

6. The process of making a propeller which consists in pressing a fibrous pulp to 85 the form of a core, electroplating said core with metal, different kinds of metal being used for coating different parts of said propeller.

In testimony whereof I have hereunto subscribed my name in the presence of two sub- 90 scribing witnesses.

MILES C. ST. JOHN.

Witnesses:

RIDSDALE ELLIS,  
CARLTON HILL.